

## UNITED STATES PATENT OFFICE

2,367,264

## BENEFICIATING LUBRICANTS, ETC.

Robert E. Burk and Everett C. Hughes, Cleveland Heights, Ohio, assignors to The Standard Oil Company, Cleveland, Ohio, a corporation of Ohio

No Drawing. Application September 30, 1940,  
Serial No. 359,095

2 Claims. (Cl. 252—47)

Various agents have been proposed for incorporation in lubricating oils and the like for restraining deterioration, some having more or less utility in such direction. We have now found that a peculiar group of organic compounds of quite complex character is of outstanding action and utility in petroleum products particularly of low volatile character.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

A lubricating stock for instance, which it is desired to protect against deterioration, as in drastic usage in an internal combustion engine, is, in accordance with the present invention, provided with a small amount of a substituted phenylmethane compound, among which the phenyl group may have substituents, or the methane carbon atom may be replaced by substituents, or substituents may occur in both. Compounds are desirable which are of the general formula



in which R is hydrogen, hydrocarbon radical or substituted derivatives of such group, or acyl residue, X is carbon, nitrogen, sulphur, S—S, oxygen, phosphorus, aluminum, boron, arsenic, antimony, O—P—O, or O—Al—O, and optionally with one or two side groups which may be hydrogen, hydrocarbon radical or derivative or substitution product, oxygen-, sulphur-, or nitrogen-derivatives, or halogen except as side group from sulphur or nitrogen. Illustrative of such compounds are Michler's hydrol or tetramethyldiaminobenzhydrol, Michler's thiohydrol, Michler's ketone, Michler's thioketone, tetramethyldiaminodiphenyl mono or dichloromethane, 4,4'-dimethylaminobenzophenonimide, aluminum tri-Michler's hydrolate, Michler's hydrolxanthate, tetramethyldiaminodiphenylamine, tetramethyldiaminodiphenyldisulphide, tetramethyldiaminodiphenylphosphine, p-diaminodiphenyldisulphide, etc. These agents are applied in amount of 0.05 to 5.0 per cent, depending upon the stock and the particular duty in view. In general, less than 2 per cent is sufficient. The agent is readily dissolved

and disseminated in the oil. The lubricating stock may be of source and character as desired, and for instance 45 to 200 sec. Saybolt Universal at 210° F.

5 Similarly such agent may be introduced into other petroleum products, such as asphalt, etc., solid products conveniently being molten to permit thorough dissemination of the agent.

As an example: With a 20 S. A. E. lubricating 10 stock of Mid-Continent source, there is incorporated 0.25 per cent of Michler's thiohydrol. This lubricant, when tested by the common quick test, viz, subjection to a temperature of 300° F. in full exposure to air bubbled through at the 15 rate of thirty liters per hour, for 65 hours, showed a viscosity increase of 57, naphtha insolubles 2.6 per cent, lacquer formation 14.0 percent, and appearance rating B minus. In contrast, the oil without the Michler's thiohydrol, similarly tested, 20 showed a viscosity increase of 236, naphtha insolubles 7.7, lacquer formation 43.3, and appearance rating D.

As another example: With a similar oil there 25 is incorporated 0.25 per cent of tetramethyldiaminobenzhydrol. This lubricant, tested as foregoing, showed a viscosity increase of 33, naphtha insolubles 0.3, lacquer formation 4.2, and appearance rating B minus.

As another example: With a similar oil there 30 is incorporated 0.25 per cent of 4,4'-dimethylaminobenzophenonimide.

As another example: With a similar oil there is incorporated 0.25 per cent of diaminodiphenyl-disulphide.

35 Particularly advantageous are the compounds of the above general formula in which X is as stated, except carbon and nitrogen.

Other modes of applying the principle of the 40 invention may be employed, change being made as regards the details described, provided the features stated in any of the following claims, or the equivalent of such, be employed.

We therefore particularly point out and distinctly claim as our invention:

45 1. A composition consisting of a normally non-volatile hydrocarbon product and a small amount of a substituted aminodiphenylmethane compound having bonded to its central carbon atom an atom of group VI of the periodic system of atomic weight not exceeding that of sulphur.

2. A normally non-volatile hydrocarbon product containing a small amount of Michler's thiohydrol.

ROBERT E. BURK.  
EVERETT C. HUGHES.